



of paratoluene-sulphonamide with one mole of cyanuryl chloride prepared according to the process described in the "Journal of the Chemical Society," 1963, page 4131, 0.5 part of crystalline ammonium acetate and 10 parts of anhydrous sodium sulphate. The temperature of the bath is brought to boiling in a period of 30 minutes, and this temperature is maintained for an hour. The temperature of the bath is then reduced to 95° C., and the pH is brought to 8 by the addition of dilute ammonia. The treatment is continued for 15 minutes. The "nylon" thread is then washed with soap and rinsed.

The thread thus treated and an untreated thread are then dyed with the dyestuff known by the name of "Rouge Ponceau Acide BL" (Colour Index "Acid Red 106". The dyestuff possesses very little affinity for the treated "nylon," while the untreated thread is dyed a bright red.

#### EXAMPLE 2

10 parts of "nylon" thread are introduced at ambient temperature into a bath containing 200 parts of water, 1 part of the sodium salt of the condensate from one mole of parachlorobenzene sulphonamide with one mole of cyanuryl chloride, 10 parts of sodium chloride and 0.2 part of sodium bicarbonate. The temperature of the bath is brought to boiling temperature in a period of 45 minutes and this temperature is maintained for one hour. The thread is washed with soap and rinsed. The behaviour of the treated "nylon" is comparable with that described in Example 1.

#### EXAMPLE 3

10 parts of "nylon" thread are introduced into a bath at 40° C. containing 300 parts of water, 0.5 part of the monosodium salt of the condensate from one mole of paratoluene sulphonamide with one mole of the chloride of 2,3-dichloroquinoxaline-6-carboxylic acid. The bath, the pH of which is regulated at 5 by the addition of 1% acetic acid, is taken to boiling temperature in a period of 30 minutes and is maintained at this temperature for 30 minutes. The temperature of the bath is then reduced to 95° C. and the pH is brought to a value of 8 by the addition of disodium phosphate, and the treatment is followed for 15 minutes. The thread is washed with soap and rinsed. The behaviour of the "nylon" towards acid dyestuffs is similar to that described in Example 1.

#### EXAMPLE 4

A printed paste is prepared containing the following components:

60 parts of the sodium salt of the condensate from one mole of paratoluene sulphonamide with one mole of cyanuryl chloride  
 60 parts of thiourea  
 500 parts of a 4% alginic acid thickener  
 20 parts of sodium acetate  
 360 parts of water  
 1000 parts

A "nylon" fabric is printed with this paste and steamed for 30 minutes at 100–102° C. It is rinsed, washed with soap, rinsed again and immersed in a dyebath containing 1 g. per litre of bath liquid of the dyestuff known as "Rouge Ponceau Acide BL." The fabric is dyed red, the printed parts remaining white.

#### EXAMPLE 5

10 parts of "nylon" thread are introduced into a bath

at 40° C. containing 200 parts of water, 1 part of the sodium salt of the condensate from one mole of paratoluene sulphonamide with one mole of cyanuryl chloride, 20 parts of anhydrous sodium sulphate, 10 parts of 1% acetic acid and 10 parts of 10% sodium acetate. The temperature of the bath is brought to boiling in the course of 30 minutes and is maintained at this temperature for one hour. The "nylon" is then treated for an hour in a second bath at 95° C. containing per litre 250 g. of sodium chloride and 65 g. of 2% ammonia, washed with soap and rinsed. The behaviour of the "nylon" towards acid dyestuffs is similar to that described in Example 1.

#### EXAMPLE 6

If in Example 5 the 2% ammonia is replaced by a 10% solution of triethanolamine, analogous results are obtained.

We claim:

1. Process for the modification of synthetic polyamide fibres which comprises treating the fibres at a pH of from 3 to 11 inclusive and at a temperature of from 40° C. to the boiling temperature of the bath with a compound of the formula:



in which  $A_1$  represents the radical of a non-colouring compound of the aliphatic, aromatic or heterocyclic series free from carboxylic and sulphonate groups,  $R$  represents a hydrogen atom or an alkyl group having 1 to 4 carbon atoms and  $W$  represents a halogenated triazinyl group, a halogenated pyrimidinyl group, the 2,4-dichloro-pyrimidine-6-carbonyl group, the 2,3-dichloroquinoxaline-5-carbonyl group, the 2,3-dichloro-quinoxaline-6-carbonyl group, the 1,4-dichloro-phthalazine-5-carbonyl group, the 1,4-dichloro-phthalazine-6-carbonyl group, the  $\beta$ -chloro-propionyl group of the acryloyl group, the compound (I) being present in the amount of between 0.1% and 20% by weight of the polyamide fibres.

2. Process according to claim 1 wherein  $A_1$  carries at least one non-auxochrome substituent.

3. Process according to claim 1 wherein the compound (I) is used in the form of an aqueous solution.

4. Process according to claim 1 wherein the compound (I) is used in the form of an aqueous dispersion.

5. Process for the modification of synthetic polyamide fibres which comprises applying thereto a printing paste containing a compound of the Formula I, in the amount of between 0.1% and 20% and steaming the printed fibres.

6. Process according to claim 1 wherein the treatment is in two stages, the first being in an acid bath containing the compound of the Formula I and the second in an alkaline bath charged with electrolyte at a pH between 7 and 11.

7. Synthetic polyamide fibers modified by a process according to claim 1.

#### References Cited

##### UNITED STATES PATENTS

3,377,336 4/1968 Siegel et al. \_\_\_\_\_ 8—1.22X

DONALD LEVY, Primary Examiner

T. J. HERBERT, JR., Assistant Examiner

U.S. CL. X.R.